# EUROPEAN PATENT SPECIFICATION

(11) **EP 2 312 007 B1**
(45) Date of publication and mention of the grant of the patent: **26.02.2014**
(21) Application number: 09804914.1
(22) Date of filing: 24.07.2009
(51) Int. Cl.: C22C 38/00, B21B 3/00, C21D 9/46, C22C 38/16, C22C 38/60

(54) **HIGH-STRENGTH COLD-ROLLED STEEL SHEET EXCELLENT IN WELDABILITY AND PROCESS FOR PRODUCTION OF SAME**
HOCHFESTES KALTGEWALZTES STAHLBLECH MIT HERVORRAGENDER SCHWEISSBARKEIT UND HERSTELLUNGSVERFAHREN DAFÜR
TÔLE D'ACIER LAMINÉE À FROID DE HAUTE RÉSISTANCE, PRÉSENTANT UNE EXCELLENTE APTITUDE AU SOUDAGE, ET SON PROCÉDÉ DE FABRICATION

(30) Priority: 05.08.2008 JP 2008201735
(43) Date of publication of application: 20.04.2011
(73) Proprietor: JFE Steel Corporation, Tokyo 100-0011 (JP)
(72) Inventor: YOSHIDA, Hiromi, Tokyo 100-0011 (JP); SAITO, Hayato, Tokyo 100-0011 (JP); YOKOTA, Takeshi, Tokyo 100-0011 (JP); TANAKA, Yasushi, Tokyo 100-0011 (JP)
(74) Representative: Grünecker, Kinkeldey, Stockmair & Schwanhäusser
(86) International application number: PCT/JP2009/063622
(87) International publication number: WO 2010/016430

(56) References cited:
- EP-A1- 0 632 141
- JP-A- 3 150 315
- JP-A- 6 100 980
- JP-A- 6 212 276
- JP-A- 7 188 772
- JP-A- 8 291 364
- JP-A- 10 183 253
- US-A- 5 156 690

## Description

### Technical Field

The present invention relates to a high strength cold rolled steel sheet with formability and weldability that is suitably used for structures such as railway vehicles, automobiles, and ships. In particular, the present invention relates to a high strength cold rolled steel sheet having a tensile strength TS of 440 MPa or more and a method for manufacturing the same.

### Background Art

With the progress of degassing technologies in a steelmaking process, it has been possible to manufacture a large amount of ultra low carbon steel whose C amount is reduced to 0.0030% or less by mass at relatively low costs. An interstitial free (IF) cold rolled steel sheet with excellent formability made by adding a carbonitride-forming element such as Ti or Nb to ultra low carbon steel has been widely used for automobile components, electric device components, and the like. Thus, various IF cold rolled steel sheets have been developed. For example, Patent Documents 1 and 2 disclose cold rolled steel sheets with excellent formability. In the cold rolled steel sheets, resistance to cold-work embrittlement is improved by further adding B to the IF steel to which Ti or Nb is added. Patent Document 3 discloses a deep-drawing steel sheet with excellent brazing property obtained by further adding Ni to the IF steel to which Ti or Nb is added.

In recent years, an automotive steel sheet having higher strength has been developed in terms of weight reduction of a car body and crash safety of automobiles. Furthermore, a tailor-welded-blank made by combining two or more steel sheets having different thicknesses and characteristics through welding has been used as an automotive steel sheet to reduce the numbers of steps and dies. Therefore, there has been a growing demand for a high strength steel sheet with excellent formability and weldability, particularly a high strength cold rolled steel sheet having a TS of 440 MPa or more.

The IF cold rolled steel sheet described above is desired in consideration of formability. However, the weldability of a tailor-welded-blank that uses an IF cold rolled steel sheet has hardly been investigated. Regarding the weldability of a tailor-welded-blank, Patent Document 4 discloses a method for manufacturing a tailor-welded-blank by welding steel sheets having different thicknesses through plasma welding that is performed with low equipment cost, at high speed, and without using a welding metal. In that method, a weld defect called humping bead is prevented by adjusting the C amount of the thicker steel sheet to 0.1% or more by mass or by adjusting the Si amount to 0.8% or more by mass.

### Related Art Documents

Patent Document 1: Japanese Unexamined Patent Application Publication No. 61-246344
Patent Document 2: Japanese Unexamined Patent Application Publication No. 1-149943
Patent Document 3: Japanese Unexamined Patent Application Publication No. 2-232342
Patent Document 4: Japanese Unexamined Patent Application Publication No. 2003-94170

### Disclosure of Invention

### Problems to be Solved by the Invention

However, in the method for manufacturing a tailor-welded-blank described in Patent Document 4, the C amount of at least one of the steel sheets needs to be adjusted to 0.1% or more by mass or the Si amount needs to be adjusted to 0.8% or more by mass. This poses a problem in that the formability of the tailor-welded-blank is significantly deteriorated.

In addition, high speed plasma arc welding easily causes the formation of humping bead. This poses a problem of high speed welding, that is, difficulty in improving productivity. To solve the problems, an object of the present invention is to achieve high speed welding by improving a steel sheet.

In other words, an object of the present invention is to provide a high strength cold rolled steel sheet with excellent weldability in which humping bead is not formed by performing plasma welding at high speed and that has a TS of 440 MPa or more, which does not deteriorate the formability of a tailor-welded-blank. Another object of the present invention is to provide a method for manufacturing the high strength cold rolled steel sheet.

### Means for Solving the Problems

The inventors of the present invention discovered the following findings after their investigation about the formability and weldability of a high strength cold rolled steel sheet in which humping bead is not formed by performing plasma welding at high speed and that has a TS of 440 MPa or more, which does not deteriorate the formability of a tailor-welded-blank.
i) The formation of humping bead during high speed plasma welding can be suppressed by adding Cu to IF steel, and further prevented by controlling the O amount in the steel within a proper range.
ii) Excellent formability of a tailor-welded-blank is achieved by adjusting the C amount to 0.005% or less by mass, by using IF steel to which Ti is added, and by using a microstructure constituted by a ferrite single phase.

Accordingly, the present invention provides a high strength cold rolled steel sheet that is excellent in weldability and has a TS of 440 MPa or more, including a composition including C: 0.0005 to 0.005%, Si: 0.1 to 1.0%, Mn: 1 to 2.5%, P: 0.01 to 0.2%, S: 0.015% or less, sol. Al: 0.05% or less, N: 0.007% or less, Ti: 0.01 to 0.1%, B: 0.0005 to 0.0020%, Cu: 0.05 to 0.5%, and Ni: 0.03 to 0.5% by mass with the balance Fe and incidental impurities; and a microstructure constituted by a ferrite single phase.

In the high strength cold rolled steel sheet of the present invention, the composition preferably further includes 0: 0.0025 to 0.0080% by mass or at least one of Se: 0.0005 to 0.01% and Te: 0.0005 to 0.01% by mass.

The high strength cold rolled steel sheet of the present invention can be manufactured by a method including the steps of hot-rolling a slab having the composition described above, coiling at a coiling temperature of 680°C or less, pickling, cold-rolling at a reduction ratio of 40% or more, and performing recrystallization annealing at 700 to 850°C.

### Advantages

According to the present invention, a high strength cold rolled steel sheet with excellent weldability in which humping bead is not formed by performing plasma welding at high speed and that has a TS of 440 MPa or more, which does not deteriorate the formability of a tailor-welded-blank can be manufactured. Furthermore, the high strength cold rolled steel sheet of the present invention with excellent formability is suitably used for not only automobile components but also electric device components and the like.

### Best Mode for Carrying Out the Invention

The present invention will now be described in detail. Herein, % denotes the amount of elements expressed as percent by mass unless specified.

### 1) Composition

### C: 0.0005 to 0.005%

When the C amount is less than 0.0005%, a heavy burden is placed on decarbonization refining at a steelmaking stage, which increases the costs due to, for example, vacuum degassing. When the C amount is more than 0.005%, the formability is deteriorated. Thus, the C amount is in the range of 0.0005 to 0.005%, and is preferably 0.003% or less.

### Si: 0.1 to 1.0%

Si is an element that is effective for imparting higher strength to steel. To achieve such an effect, the Si amount needs to be 0.1% or more. However, a Si amount of more than 1.0% causes embrittlement of ferrite, which impairs the strength-ductility balance. Thus, the Si amount is in the range of 0.1 to 1.0%, and is preferably 0.7% or less.

### Mn: 1 to 2.5%

Mn is an element that is effective for imparting higher strength to steel. To achieve such an effect, the Mn amount needs to be 1% or more. However, a Mn amount of more than 2.5% facilitates centerline segregation in a slab and deteriorates the formability of end products. Thus, the Mn amount is in the range of 1 to 2.5%. To prevent hot brittleness due to FeS formation, Mn is combined with solid solution S in the steel to form MnS. In this case, assuming that the Mn amount is [Mn] and the S amount is [S], it is preferable to satisfy ([Mn]/55)/([S]/32) > 100.

### P: 0.01 to 0.2%

P is an element that is effective for imparting higher strength to steel. To achieve such an effect, the P amount needs to be 0.01% or more. However, a P amount of more than 0.2% not only may cause grain boundary fracture in an HAZ or deteriorates low temperature toughness of a base metal or a welded portion, but also deteriorates an anti-crash property due to grain boundary segregation. Thus, the P amount is in the range of 0.01 to 0.2%.

### S: 0.015% or less

A S amount of more than 0.015% deteriorates low temperature toughness of a base metal or a welded portion as with P. Thus, the S amount is 0.015% or less, and a smaller amount is preferable. As described above, it is preferable to satisfy ([Mn]/55)/([S]/32) > 100.

### sol. Al: 0.05% or less

Al is normally used as a deoxidizing element at a steelmaking stage. Since the 0 amount is controlled within a specific range in the present invention, the sol. Al amount is 0.05% or less. A sol. Al amount of more than 0.05% is not preferable because the formability is deteriorated due to a large amount of Al₂O₃ and inclusions may cause weld cracking. Thus, the sol. Al amount is 0.05% or less.

### N: 0.007% or less

A N amount of more than 0.007% deteriorates the formability and anti-aging property. Thus, the N amount is 0.007% or less, and a smaller amount is preferable.

### Ti: 0.01 to 0.1%

Ti improves the formability and anti-aging property by forming a precipitate with C or N. To achieve such an effect, the Ti amount needs to be 0.01% or more. However, a Ti amount of more than 0.1% increases an alloy cost. Thus, the Ti amount is in the range of 0.01 to 0.1%. To effectively produce the effect of B described below, assuming that the Ti amount is [Ti] and the N amount is [N], it is preferable to satisfy [N] - (14/48)[Ti] ≤ 0.

### B: 0.0005 to 0.0020%

B improves the resistance to cold-work embrittlement when B exists in a solid solution state. To achieve such an effect, the B amount needs to be 0.0005% or more. However, a B amount of more than 0.0020% facilitates weld cracking. Thus, the B amount is in the range of 0.0005 to 0.0020%.

### Cu: 0.05 to 0.5%

Cu is an element that is effective for imparting higher strength without deteriorating formability and for preventing the formation of humping bead during high speed plasma welding. In particular, the effects are increased when Cu coexists with O controlled within the range described below in the steel. To achieve such effects, the Cu amount needs to be 0.05% or more.

However, a Cu amount of more than 0.5% saturates the effects and significantly deteriorates surface quality. Thus, the Cu amount is in the range of 0.05 to 0.5%. The reason why the formation of humping bead during high speed plasma welding can be prevented when Cu coexists with 0 is uncertain, but it is believed that the viscosity of the steel melted during welding is optimized, which improves the flowability of molten steel.

### Ni: 0.03 to 0.5%

The content of Cu described above easily deteriorates surface quality. To prevent it, a Ni amount of 0.03% or more needs to be added. However, a Ni amount of more than 0.5% saturates the effect. Thus, the Ni amount is in the range of 0.03 to 0.5%. Assuming that the Ni amount is [Ni] and the Cu amount is [Cu], it is preferable to satisfy 0.25 × [Cu] ≤ [Ni] ≤ 0.75 × [Cu].

Although the balance is Fe and incidental impurities, 0: 0.0025 to 0.0080% or at least one of Se: 0.0005 to 0.01% and Te: 0.0005 to 0.01% is preferably further contained because of the following reasons.

### O: 0.0025 to 0.0080%

As described above, the formation of humping bead during high speed plasma welding can be further suppressed when 0 coexists with Cu. It is believed that the viscosity and surface tension of the molten steel during welding is further optimized when O coexists with Cu. To achieve such an effect, the 0 amount in the steel needs to be 0.0025% or more, preferably 0.0040% or more. However, an 0 amount of more than 0.0080% saturates the effect, increases the cost for treating a slab surface due to a large number of blowholes of a continuous casting slab, and deteriorates the formability of the steel because of an increase in the number of inclusions.

### Se: 0.0005 to 0.01% and Te: 0.0005 to 0.01%

As with 0, Se and Te optimize the viscosity and surface tension of the molten steel during welding and prevent the formation of humping bead during high speed plasma welding when they coexist with Cu. To achieve such effects, the Se or Te amount needs to be 0.0005% or more. However, a Se or Te amount of more than 0.01% saturates the effects.

### 2) Microstructure

In terms of formability, a microstructure constituted by a ferrite single phase is required. The ferrite single phase herein may be either a polygonal ferrite phase or a bainitic ferrite phase or a mixture thereof. To ensure a TS of 440 MPa and prevent the excessive softening of a welded portion, the average grain diameter of the ferrite phase is preferably 50 µm or less.

### 3) Manufacturing Conditions

The high strength cold rolled steel sheet of the present invention can be manufactured by a method including the steps of hot-rolling a slab having the composition described above, coiling at a coiling temperature of 680°C or less, pickling, cold-rolling at a reduction ratio of 40% or more, and performing recrystallization annealing at 700 to 850°C.
Coiling Temperature after Hot Rolling: 680°C or less

When the coiling temperature is more than 680°C, a chemical compound of P and Fe, Ti, or the like is easily formed, which impedes the development of a {111} texture that is preferred for deep-drawing formability when cold-rolling and annealing performed later. Thus, the coiling temperature is 680°C or less, preferably 650°C or less.
Reduction Ratio of Cold Rolling: 40% or more

In terms of formability, the reduction ratio is 40% or more. In terms of improvement in formability and, particularly, deep drawability, the reduction ratio is preferably 50% or more.
Recrystallization Annealing Temperature: 700 to 850°C

The annealing temperature needs to be 700°C or more for recrystallization. However, when the annealing temperature exceeds 850°C, ferrite grains are coarsened, which decreases strength or deteriorates surface quality. Thus, the recrystallization annealing temperature is in the range of 700 to 850°C. To sufficiently perform recrystallization, a steel sheet is preferably held at 750°C or more for 30 seconds or longer.

Manufacturing conditions of typical methods can be applied to other manufacturing conditions of the present invention. In other words, steel is smelted in a converter or an electric furnace to form a slab through continuous casting. For hot rolling, the slab may be rolled after heat treatment, directly rolled without heat treatment, or rolled after short-time heat treatment. Hot rolling may be performed at a finishing temperature equal to or higher than the Ar₃ transformation temperature as with typical procedures. The recrystallization annealing can be performed by box annealing or continuous annealing. After the annealing, skin pass rolling may be performed, for example, for the purpose of the adjustment of surface roughness and the planarization of a plate shape. Subsequently, surface treatments such as a chemical conversion treatment and a plating treatment may be conducted.

### Example 1

Each of steel Nos. 1 to 7 having an elemental composition of 0:002% C-0.2% Si-1.8% Mn-0.05% P-0.005% S-0.02% sol. Al-0.003% N-0.04% Ti-0.0010% B with Cu, 0, and Se shown in Table 1 was smelted by vacuum melting, heated at 1200°C for 1 hour, and then rough-rolled to make a sheet bar having a thickness of 35 mm. The sheet bar was heated at 1250°C for 1 hour and finish-rolled such that the finish rolling entering temperature was 900°C after seven passes. Subsequently, heat treatment corresponding to coiling was performed at 580°C for 1 hour to obtain a hot rolled steel sheet having a thickness of 4 mm. The hot rolled steel sheet was descaled through pickling and cold-rolled at a reduction ratio of 60% to obtain a cold rolled steel sheet having a thickness of 1.6 mm. Recrystallization annealing in which heating is conducted at 830°C for 180 sec and cooling is then conducted at a cooling rate of 10°C/sec was performed using a salt bath. After pickling was performed in order to remove the salt attached to the surface of the steel sheet, skin pass rolling was conducted at an elongation percentage of 0.5%.

Steel sheets having the same composition were plasma-welded at a welding speed of 0.2 to 1.4 m/min under the following fixed conditions to investigate the "presence" or "absence" of humping bead: welding current: 60A, Ar gas flow rate for plasma: 0.6 L/min, Ar gas flow rate for shield: 10 L/min, nozzle size: 2.0 mmφ, and nozzle-sample distance: 3 mm.

Table 1 shows the results.

In the existing plasma welding, the maximum speed that can achieve welding without forming humping bead was about 0.2 to 0.4 m/min. In contrast, humping bead was not formed at a high welding speed of 1 m/min in the sample (steel No. 3) containing Cu according to the present invention and at a high welding speed of 1 m/min or more in the samples (steel Nos. 4 to 7) further containing 0 and Se. Accordingly, the samples of the present invention have high speed plasma weldability.

**Table 1**

| Steel No. | Cu (% by mass) | Ni (% by mass) | O (% by mass) | Se (% by mass) | Welding speed (m/min) and Humping bead presence (×) absence (○) | | | | | | |
|---|---|---|---|---|---|---|---|---|---|---|---|
| | | | | | 0.2 | 0.4 | 0.6 | 0.8 | 1.0 | 1.2 | 1.4 |
| 1 | 0 | 0 | <0.002 | 0 | ○ | × | | | | | |
| 2 | 0.01 | 0.05 | <0.002 | 0 | ○ | ○ | × | | | | |
| 3 | 0.05 | 0.03 | <0.002 | 0 | ○ | ○ | ○ | ○ | ○ | × | |
| 4 | 0.05 | 0.03 | 0.0040 | 0 | ○ | ○ | ○ | ○ | ○ | ○ | |
| 5 | 0.1 | 0.05 | 0.0030 | 0 | ○ | ○ | ○ | ○ | ○ | ○ | |
| 6 | 0.1 | 0.05 | 0.0050 | 0 | ○ | ○ | ○ | ○ | ○ | ○ | ○ |
| 7 | 0.1 | 0.05 | 0.0030 | 0.0010 | ○ | ○ | ○ | ○ | ○ | ○ | ○ |

### Example 2

Each of steel Nos. A to F having compositions shown in Table 2 was smelted to obtain a slab through continuous casting. The slab was heated at 1200°C and then finish-rolled at a finishing temperature of 900°C. The slab was coiled at a coiling temperature of 580°C to obtain hot rolled steel sheets having thicknesses of 6 mm and 4 mm. The hot rolled steel sheets were pickled and cold-rolled at a reduction ratio of 60% to obtain cold rolled steel sheets having thicknesses of 2.4 mm and 1.6 mm. Continuous annealing was performed at an annealing temperature of 830°C and skin pass rolling was conducted at an elongation percentage of 0.5%.

Steel sheets having the same composition were plasma-welded in accordance with the combinations of sheet thickness shown in Table 3 under the following fixed conditions to investigate the "presence" or "absence" of humping bead: welding current: 60A, Ar gas flow rate for plasma: 0.6 L/min, Ar gas flow rate for shield: 10 L/min, nozzle size: 2.0 mmφ, nozzle-sample distance: 3 mm, and welding speed: 1 m/min. Furthermore, TS and total elongation El in a direction perpendicular to the rolled direction of the obtained steel sheets and an average r value were measured using JIS 5 test pieces.

Table 3 shows the results. The steel sheets having compositions of invention examples exhibit a TS of 440 MPa or more and are excellent in formability. For the steel sheets, humping bead is not formed during high speed plasma welding.

**Table 2**

| Steel No. | Composition (% by mass) | | | | | | | | | | | | | | Note |
|---|---|---|---|---|---|---|---|---|---|---|---|---|---|---|---|
| | C | Si | Mn | P | S | sol.Al | N | Ti | B | Cu | Ni | O | (Mn/55)/(S/32) | Other | |
| A | 0.0015 | 0.2 | 1.9 | 0.079 | 0.007 | 0.050 | 0.0016 | 0.037 | 0.001 | 0.09 | 0.05 | <0.002 | 158 | - | within the scope of the invention |
| B | 0.0025 | 0.2 | 2.0 | 0.075 | 0.007 | 0.050 | 0.0015 | 0.035 | 0.0015 | 0.12 | 0.05 | 0.005 | 166 | - | within the scope of the invention |
| C | 0.0015 | 0.7 | 1.2 | 0.030 | 0.006 | 0.030 | 0.0020 | 0.061 | 0.0015 | 0.06 | 0.035 | 0.003 | 116 | Se:0.005 | within the scope of the invention |
| D | 0.0012 | 0.6 | 1.3 | 0.036 | 0.008 | 0.026 | 0.0007 | 0.032 | 0.0006 | 0 | 0.06 | <0.002 | 95 | - | outside the scope of the invention |
| E | 0.0015 | 0.5 | 0.8 | 0.030 | 0.007 | 0.030 | 0.0020 | 0.06 | 0.0015 | 0.15 | 0.080 | 0.005 | 66 | - | outside the scope of the invention |
| F | 0.0015 | 0.1 | 0.3 | 0.075 | 0.003 | 0.050 | 0.0015 | 0.035 | 0.0015 | 0.1 | 0.05 | 0.007 | 58 | - | outside the scope of the invention |

**Table 3**

| Steel No. | Combination of sheet thickness | TS (MPa) | El (%) | Average r value | Humping bead presence (×) absence (○) | Note |
|---|---|---|---|---|---|---|
| A | 1.6/1.6 | 450 | 40 | 1.6 | ○ | Invention Example |
| B | 1.6/1.6 | 510 | 35 | 1.4 | ○ | Invention Example |
| | 2.4/1.6 | 510 | | | ○ | Invention Example |
| C | 2.4/1.6 | 470 | 38 | 1.5 | ○ | Invention Example |
| D | 1.6/1.6 | 480 | 38 | 1.5 | × | Comparative Example |
| E | 1.6/1.6 | 420 | 43 | 1.4 | ○ | Comparative Example |
| F | 1.6/1.6 | 285 | 60 | 1.8 | ○ | Comparative Example |

| | | | | | | |
|---|---|---|---|---|---|---|
| TS, El, and r value are material property values in 1.6 mmt | | | | | | |

## Claims

1. A high strength cold rolled steel sheet that is excellent in weldability and has a tensile strength of 440 MPa or more, comprising a composition consisting of C: 0.0005 to 0.005%, Si: 0.1 to 1.0%, Mn: 1 to 2.5%, P: 0.01 to 0.2%, S: 0.015% or less, sol. Al: 0.05% or less, N: 0.007% or less, Ti: 0.01 to 0.1%, B: 0.0005 to 0.0020%, Cu: 0.05 to 0.5%, and Ni: 0.03 to 0.5% and optionally 0: 0.0025 to 0.0080% and further optionally at least one of Se: 0.0005 to 0.01% and Te: 0.0005 to 0.01% by mass with the balance Fe and incidental impurities; and a microstructure constituted by a ferrite single phase.

2. A method for manufacturing a high strength cold rolled steel sheet that is excellent in weldability and has a tensile strength of 440 MPa or more, comprising the steps of hot-rolling a slab having the composition defined in Claim 1, coiling at a coiling temperature of 680°C or less, pickling, cold-rolling at a reduction ratio of 40% or more, and performing recrystallization annealing at 700 to 850°C.

## Patentansprüche

1. Hochfestes kaltgewalztes Stahlblech, das eine hervorragende Schweißbarkeit und eine Zugfestigkeit von 440 MPa oder mehr, eine Zusammensetzung bestehend aus 0,0005 bis 0,005 Massenprozent C, 0,1 bis 1,0 Massenprozent Si, 1 bis 2,5 Massenprozent Mn, 0,01 bis 0,2 Massenprozent P, 0,015 oder weniger Massenprozent S, 0,05 Massenprozent oder weniger sol. Al, 0,007 Massenprozent oder weniger N, 0,01 bis 0,1 Massenprozent Ti, 0,0005 bis 0,0020 Massenprozent B, 0,05 bis 0,5 Massenprozent Cu und 0,03 bis 0,5 Massenprozent Ni sowie ansonsten Fe und zufällige Verunreinigungen und optional 0,0025 bis 0,0080 Massenprozent O und weiterhin optional 0,0005 bis 0,01 Massenprozent Se und/oder 0,0005 bis 0,01 Massenprozent Te und eine durch ein einphasiges Ferrit gebildete Mikrostruktur aufweist.

2. Verfahren zum Herstellen eines hochfesten kaltgewalzten Stahlblechs, das eine hervorragende Schweißbarkeit und eine Zugfestigkeit von 440 MPa oder mehr aufweist, wobei das Verfahren Schritte zum Heißwalzen einer Platte mit einer Zusammensetzung wie in Anspruch 1 beschrieben, zum Wickeln bei einer Wickeltemperatur von 680°C oder weniger, zum Beizen, zum Kaltwalzen mit einem Reduktionsverhältnis von 40% oder mehr und zum Durchführen eines Rekristallisationsglühens bei 700 bis 850°C umfasst.

## Revendications

1. Tôle d'acier laminé à froid de haute résistance d'une excellente aptitude au soudage et ayant une résistance à la traction supérieure ou égale à 440 MPa, comprenant une composition constituée de C : de 0,0005 à 0,005 %, Si : de 0,1 à 1,0 %, Mn : de 1 à 2,5 %, P : de 0,01 à 0,2 %, S : 0,015 % ou moins, sol. Al : 0,05 % ou moins, N : 0,007 % ou moins, Ti : de 0,01 à 0,1 %, B : de 0,0005 à 0,0020 %, Cu : de 0,05 à 0,5 %, et Ni : de 0,03 à 0,5 % optionnel O : de 0,0025 à 0,0080 % et en outre au moins un élément parmi Se : de 0,0005 à 0,01 % et Te : de 0,0005 à 0,01 % en masse, et le complément en Fe et en impuretés accidentelles ; et une microstructure constituée d'une phase unique de ferrite.

2. Procédé de fabrication d'une tôle d'acier laminé à froid de haute résistance d'une excellente aptitude au soudage et ayant une résistance à la traction supérieure ou égale à 440 MPa, comprenant les étapes consistant à laminer à chaud une brame ayant la composition décrite dans la revendication 1, enrouler à une température d'enroulement inférieure ou égale à 680 °C, décaper, laminer à froid avec un rapport de réduction supérieure ou égale à 40 % et effectuer un recuit de recristallisation entre 700 et 850 °C.
